

April 6, 1926.

1,579,628

O. BERG ET AL

PROCESS OF WEIGHTING FIBERS AND THE PRODUCT THEREOF

Filed Dec. 26, 1922

Fig. 1



Fig. 2



INVENTOR  
Olov Berg  
Max Imhoff  
BY  
C. W. Marshall  
ATTORNEY

## UNITED STATES PATENT OFFICE.

OLAV BERG, OF PATERSON, AND MAX IMHOFF, OF CLIFTON, NEW JERSEY.

## PROCESS OF WEIGHTING FIBERS AND THE PRODUCT THEREOF.

Application filed December 26, 1922. Serial No. 609,082.

*To all whom it may concern:*

Be it known that we, OLAV BERG, a citizen of Norway, and a resident of Paterson, Passaic County, and State of New Jersey, and MAX IMHOFF, a citizen of the United States, and a resident of Clifton, Passaic County, and State of New Jersey, have invented certain new and useful Improvements in a Process of Weighting Fibers and the Product Thereof, of which the following is a specification.

This invention relates to the weighting of fibers in general, but more particularly to the weighting of silk; "weighting" being the term of the art for a process of increasing the size and weight of fiber. While the present process is particularly intended for the treatment of natural silk, it is not limited thereto.

Under methods now in vogue and employed in the past, salts of tin, iron, and to a very limited extent, of bismuth and aluminum, have been recognized as the only metal salts which could be used in a practical commercial way for the weighting of silk. Of these, only the salts of tin and iron have been employed generally; and iron only in the case of black or dark colored goods. Heretofore, the extent of weighting has been limited because after a certain amount of weighting material has been taken up, the fiber is injuriously affected. There is a practical limit in the prior art processes to the amount of mineral matter which the fiber will take up without injuring its physical properties. Usually the result was a compromise between increase in quantity and decrease in quality. While by such known processes it has been possible to add ten percent up to one hundred and thirty percent above pari, above ten percent the effect on the fibers is markedly injurious, taking away both elasticity and strength and making them brittle and tender and subject to deterioration with age. While the amount of loading permissible in producing commercial silk without undue forfeiture of quality varies with the silk and with the operator, twenty-five per cent is often considered a practical limit.

The purposes of the present invention are to improve upon former methods and to provide an inexpensive and simple method by which it is possible to weight silk or other fibers to any desired extent not only without materially impairing or destroying the

essential or desirable qualities thereof, but in fact improving them. Another object is to provide a new material produced by this process; a material which, in the best embodiment of our invention now known to us, is a fiber possessing all the textile qualities of silk but in which silk substance may be only a minor fraction; the major being composed of tin and lead oxides and  $P_2O_5$  (phosphoric acid) in some form of combination with each other and with the silk substance. The result is a sort of composite fiber which, although silky, flexible and strong, and homogeneous under the microscope, is nevertheless largely mineral matter.

The lead in the fiber is fixedly held and is insoluble. The new fiber, although containing in some embodiments as high as two hundred per cent weighting, largely  $PbO$ , does not yield lead to boiling vinegar (three per cent acetic acid) or to any of the liquids with which silk is likely to come in contact in the dye-house or in use.

One phase of the invention relates to the discovery of a method by which there is created in the silk, an affinity for lead compounds, making it possible to combine lead compounds with the fibers in such a way as to materially increase its weight and the size of the fiber; that is, so as to give a composite fiber in which a large fraction of the fiber is lead in some form; this composite fiber having the desirable properties of ordinary weighted silk without its usual disadvantages and having certain new and useful advantages of its own. In this method the silk or other fibrous material is first treated with a substance which the fibers readily take up and which gives the fibers the ability to take up lead compounds after which the latter material is added, for instance, in the form of an organic salt in solution, such as lead acetate. So to speak, the fiber is "mordanted" with materials giving it an affinity for lead.

For purposes of disclosure, we have illustrated in the accompanying drawing, in diagrammatic fashion, how the various steps of the invention may be performed; wherein, Fig. 1 indicates the preliminary weighting and preparational steps and in which Fig. 2 indicates the subsequent weighting steps.

A special feature of the preliminary or primary weighting operations, by which the affinity for the heavier metallic compounds, is created, is that they may be the same as

heretofore have been employed in tin-weighting and like processes, so that the apparatus and the materials now at hand may be employed. The usual solutions used in weighting with tin may be employed as a first bath, namely, a solution of tin tetrachloride (stannic chloride) or of "pink salt", which is a combination of tin tetrachloride and ammonium chloride. A solution of sodium 10 stannate has been used in tin weighting. So have potassium or ammonium stannates been used but are not better than sodium stannate. Any of these materials used in aqueous solution deposit on the silk a certain amount 15 of tin in a form equivalent to stannic oxide,  $\text{SnO}_2$ .

Thus in Fig. 1 the fibrous material, which in the case of silk may be either in the gum, de-gummed or partially de-gummed condition and may be in the form of fibers, or woven or knitted fabric, is shown at 5 as passing first into a bath 6 of a solution of stannic chloride, ( $\text{SnCl}_4$ ), then through a wash at 7 of water, then into a fixing bath at 25 8, such as of sodium phosphate, ( $\text{Na}_2\text{HPO}_4 \cdot 12\text{H}_2\text{O}$ ), followed by another water wash at 9. In the first bath, which may be a cold one, as well known, a certain amount of weight is added to the fiber and excess material, stannic chloride and  $\text{HCl}$ , is removed in the first water wash, (which also may be cold), the latter also apparently having to some extent a hydrolyzing effect on the tin chloride remaining in the fiber; breaking it 30 up in a way equivalent to the production of tin oxide remaining with the fiber and hydrochloric acid which goes off with the water.

In place of sodium phosphate other alkaline salts or carbonates may be used in what we have termed the fixing bath at 8, the temperature of this bath being such as that heretofore used in the art. In using a phosphate bath, a large amount of  $\text{P}_2\text{O}_5$  is taken 40 up. As far as our present knowledge goes, sodium phosphate is the best substance to use. In the weighting and fixing baths, the weight is increased, usually, about ten percent. The wash following the fixing bath 45 may be either cold or warm. These steps are old and well known in the art and may be and usually are repeated a number of times. These old and well known steps constitute the first stage of our complete 50 process and are designated in the drawings as the "A" stage.

The next stage in the process may be either that shown at B or that shown at C in the drawings. The stage shown at B is 60 a bath at 10 of aluminum sulphate followed by a water wash at 11. If this is used, it adds further weight to the treated material; the accession in weight being due to the taking up of  $\text{Al}_2\text{O}_3$ . The stage designated by 65 C in the drawings is a bath of water-glass

at 12 followed by a water wash at 13. This stage also adds to the weight of the treated material;  $\text{SiO}_2$  being taken up.

The stage B or the stage C follow after the stage A has been repeated as many times as desired. Sometimes both of the stages B and C are utilized after the desired treatment by the stage A, but as far as our process is concerned, the new steps, which we are about to describe as the D stage, may follow directly after the A stage treatment, after the B stage treatment or after the C stage treatment, (in the latter case whether or not the B stage treatment has been used). While our discovery is in the D stage treatments, preparation of the silk is required for the use of the D stage, and our process therefore comprises some steps preliminary to the D stage. These preliminary steps may be, as stated, the old and well known operations used in weighting silk. 80

We have discovered that the A stage treatment, weighting the fibers with tin salts and fixing them, imparts to the fiber thus treated an affinity for other metallic compounds. We have found that the fibers can be further weighted to practically any desired extent by subjecting them to the treatment illustrated diagrammatically in Fig. 2. In the best embodiment of our invention at present known to us, the further weighting is done with the aid of lead compounds, using any suitable soluble lead salt, generally lead acetate. 95

It is possible to use lead salts for this purpose because of the fact that the preparatory treatments described create in the material the property of taking up lead ( $\text{PbO}$ ) from them. In the embodiment of our invention herein shown and described, we use 100 at 14 a warm solution of lead acetate, which may be commercial sugar of lead or a more basic acetate. This, followed by a water wash at 15, is the D stage of treatment. This D stage increases the weight of the material usually from 20 per cent to 75 per 105 cent, depending upon the amount of added materials already in the fiber. The lead acetate furnishes lead which combines or unites with the associated fiber and mineral matters and forms an insoluble compound. The process may terminate here. 110

We prefer to follow this treatment by the E stage, shown diagrammatically, which is subjecting the fibers to a warm bath at 16 containing sodium phosphate, and then giving the fiber a water wash at 17. Sodium phosphate is the best salt to use at this stage. A treatment with sodium phosphate much improves the fiber prepared by the present process as so far described. This E stage not only improves the appearance and the scroop of the fiber, but imparts to it the property of being able to take up more lead compounds if it is again submerged in the 115 120 125 130

lead acetate solution at 14. Thus the D stage may be repeated after the E stage,— again and again, if desired. The permanency with which the lead is held in the fiber is increased by this phosphate after-treatment.

By thus alternately adding weight and creating an affinity or avidity for further weighting material, it is possible to add to 10 the weight of the fiber at an increasing rate to an extent greatly in excess of what has been possible heretofore.

Whether or not the aluminum sulphate or the sodium silicate treatments (B and C) 15 have been employed up to this point, either or both may be used for the purpose of a final weighting and fixing treatment. Moreover, these B and C treatments impart to the fiber a further affinity or avidity for the 20 taking up of more lead salts.

As a concrete example, we have found that with a silk treated with three applications of the tin and the phosphate, (the A stage treatment), one hundred pounds of 25 de-gummed silk fiber which in this stage had added thirty pounds in weight, with a single treatment by lead acetate and sodium phosphate (the D and E stages) took on an additional sixty-five pounds in weight; a 30 second lead acetate treatment (the D stage) added approximately fifty pounds in weight and with the affinity or avidity for the lead salts further increased by the sodium phosphate treatment, (the E stage), an additional sixty pounds in weight was added by 35 a third treatment with the lead acetate (the D stage). Another bath in sodium phosphate after this put the treated fiber in condition to take up about seventy pounds more 40 weight from another bath of lead acetate.

In the present process the weight may be further increased, after the D and E stages have been repeated as many times as desired, by giving the treated fiber another water-glass bath (the C stage). Such a bath also 45 has the effect of giving the material a still further affinity for more lead compounds.

The process may be carried on so as to 50 produce practically any desired increase in weight with the important advantage of effecting increases in weight not only without injuring the material or causing any substantial deterioration in the mechanical properties or appearance of the fiber either 55 immediately, in subsequent use or from age, but with some actual improvement in these respects. The fibers retain their flexibility and strength, as well as their appearance and their ability to take on dyes or be otherwise treated. Dyeing is more even and better and the elasticity is increased. The 60 weighted material, furthermore, has good lasting and wearing qualities, the desired scroop, is non-poisonous, and is insoluble.

65 Another important advantage of the in-

vention is that this improved lead-weighting process is applicable to such goods as are already manufactured so that a manufacturer may make one quality of goods, for example by spinning or weaving, and by giving such goods different amounts of weight by this process, may make them into any desired number of different grades by weight. Furthermore, a new and useful material is made by this process.

The drawing and description which we have made of this invention are for illustrative purposes only as we realize that many variations in the steps and the chemicals employed may be used without departing from the scope of the invention, therefore we intend no limitations other than those imposed by the appended claims. In the claims we have not included the water washing steps as it is understood from this disclosure that these follow each bath treatment.

What we claim is:

1. The process of weighting fiber which comprises preliminarily weighting the fiber with tin by any known method which includes the use of a fixing bath, and thereafter treating the fiber with a soluble lead compound.

2. The process of weighting fiber which comprises preliminarily weighting the fiber with tin by any known method which includes the use of a fixing bath, then treating the fiber with a soluble lead compound, and thereafter treating the fiber with a fixing bath.

3. The process of weighting fiber which comprises treating the fiber with a solution of a soluble tin compound and treating the same with a fixing bath, to render the treated fiber capable of taking up a lead compound, and thereafter treating the fiber with a soluble lead compound.

4. The process of weighting fiber which comprises treating the fiber with a solution of a soluble tin compound, treating the same with a soluble phosphate and thereafter treating the same with a soluble lead compound.

5. The process of weighting fiber which comprises treating the fiber with a solution of a soluble tin compound and treating the same with a fixing bath, to render the treated fiber capable of taking up a lead compound, and thereafter treating the fiber with a soluble lead compound, then treating the fiber with a soluble phosphate and again treating it with a soluble lead compound.

6. The process of weighting fiber which comprises treating the fiber with a solution of a tin compound and treating the same with a soluble phosphate, to render it capable of taking up a lead compound and thereafter treating it with a soluble lead com-

- 5 pound, then treating it with a soluble phosphate and again treating it with a soluble lead compound.
7. The process of weighting fiber which 5 comprises treating the fiber with soluble tin compounds and soluble lead compounds successively with one or more intercalated treatments with solutions of other weight giving compounds.
- 10 8. The process of weighting fiber which comprises mordanting the fiber with a tin compound and thereafter subjecting it to the alternate action of baths which contain a soluble lead compound and which contain 15 a soluble phosphate.
9. The process of weighting fiber which comprises mordanting the fiber with tin salts, and thereafter subjecting it to repeated successive treatments with sodium 20 phosphate and lead acetate baths.
10. The process of weighting fiber which comprises treating the fiber with a solution of a soluble tin compound and treating the same with a fixing bath, to render the treated fiber capable of taking up a lead compound, treating the fiber with a soluble lead compound, then treating the fiber with a soluble phosphate and then treating the fiber with a water-glass bath.
- 25 11. The process of weighting fiber which comprises forming in the fiber compounds containing tin and containing phosphorus to render the same capable of taking up a lead compound, and thereafter treating it with 30 a soluble lead compound.
12. The process of weighting fiber which comprises forming in the fiber compounds containing tin and containing phosphorus to render the same capable of taking up a lead compound, treating it with a soluble lead compound and thereafter treating it with a fixing bath.
- 40 13. The process of weighting fiber which comprises forming in the fiber compounds containing tin and containing phosphorus to render the same capable of taking up a lead compound, treating it with a soluble lead compound and thereafter treating it with a soluble phosphate and then treating 45 it with a water-glass bath.
- 50 14. The process of weighting fiber which comprises forming in the fiber compounds containing tin and containing phosphorus to render the same capable of taking up a lead compound, and thereafter treating it with a soluble lead compound, then treating it with a soluble phosphate, and again treating it with a soluble lead compound, followed by another phosphate treatment, 55 and thereafter treating it with a water-glass bath.
- 60 15. The process of weighting fiber which comprises treating the fiber with a solution of a tin compound and treating the same
- with a fixing bath, to render the treated fiber 65 capable of taking up a lead compound, treating it with a soluble lead compound, then treating it with a soluble phosphate and again treating it with a soluble lead compound, followed by a phosphate treatment, 70 and thereafter treating it with a water-glass bath.
16. The process of weighting fiber which comprises mordanting the fiber with a tin compound, thereafter subjecting it to the alternate action of baths which contain a soluble lead compound and which contain a soluble phosphate, and thereafter treating it with a water-glass bath.
17. The process of weighting fiber which 80 comprises treating a fiber which contains tin in fixed and insoluble form with a soluble lead compound.
18. A textile fiber containing tin and lead compounds in fixed and insoluble form.
- 85 19. A textile fiber of which at least fifty per cent is tin and lead compounds in fixed and insoluble form.
20. A textile fiber containing compounds of tin, lead and phosphorus.
- 90 21. A textile fiber containing tin, lead and phosphorus in fixed and insoluble form.
22. A textile fiber of which at least fifty per cent is tin, lead and phosphorus in fixed and insoluble form.
- 95 23. A textile fiber containing substantial amounts of lead in oxidized colorless form, said fiber possessing flexibility, resilience and textile strength, and said lead being irremovable by the action of warm acetic acid in strength up to five per cent.
- 100 24. A textile fiber containing substantial amounts of tin and of lead in oxidized colorless form, said fiber possessing flexibility, resilience and textile strength, and said lead being irremovable by the action of warm acetic acid in strength up to five per cent.
- 105 25. A textile fiber containing substantial amounts of tin and of lead and of phosphorus in oxidized colorless forms, said fiber possessing textile properties and said phosphorus and said lead being irremovable by the action of warm acetic acid in strength up to five per cent.
- 110 26. A textile fiber comprising natural silk containing substantial amounts of tin and of lead in oxidized colorless form, said fiber possessing flexibility, resilience and textile strength, and said lead being irremovable by the action of warm acetic acid in strength up to five per cent.
- In witness whereof, I have hereunto set my hand this 21<sup>st</sup> day of December, 1922.
- OLAV BERG.
- In witness whereof, I have hereunto set my hand this 21<sup>st</sup> day of December, 1922.
- MAX IMHOFF.